# EUROPEAN PATENT SPECIFICATION

(11) **EP 2 228 428 B1**
(45) Date of publication and mention of the grant of the patent: **16.01.2013**
(21) Application number: 10154198.5
(22) Date of filing: 22.02.2010
(51) Int. Cl.: C11D 3/37, C11D 3/08, C11D 3/10, C11D 7/12, C11D 7/14

(54) **Scale-reducing additive for automatic dishwashing systems**
Wassersteinreduzierendes Additiv für automatische Geschirrspülsysteme
Additif de réduction de tartre pour systèmes de lavage automatique de la vaisselle

(30) Priority: 13.03.2009 US 210025 P; 02.02.2010 US 337300 P
(43) Date of publication of application: 15.09.2010
(73) Proprietor: Rohm and Haas Company, Philadelphia, Pennsylvania 19106-2399 (US)
(72) Inventor: Creamer, Marianne P., Warrington PA 18976 (US); Shulman, Jan Edward, Newtown PA 18940 (US); Manna, Joseph, Quakertown PA 18951 (US)
(74) Representative: Buckley, Guy Julian

(56) References cited:
- EP-A1- 2 130 898
- EP-A2- 0 770 673
- WO-A1-01/72941
- WO-A1-03/042347
- DE-A1- 3 743 739
- US-A- 5 273 675

## Description

### Background

This invention relates generally to a formulation that minimizes mixed inorganic deposits in non-phosphate automatic dishwashing systems.

Automatic dishwashing detergents are generally recognized as a class of detergent compositions distinct from those used for fabric washing or water treatment. Automatic dishwashing detergents are required to produce a spotless and film-free appearance on washed items after a complete cleaning cycle. Phosphate-free compositions rely on non-phosphate builders, such as salts of citrate, carbonate, silicate, disilicate, bicarbonate, aminocarboxylates and others to sequester calcium and magnesium from hard water, and upon drying, leave an insoluble visible deposit. Polymers made from acrylic acid, maleic acid and 2-acrylamido-2-methylpropanesulfonic acid (AMPS) are known for use in inhibiting the scale or other insoluble deposits produced from non-phosphate builders. For example, U.S. Pat. No. 5,273,675 discloses a polymer made from acrylic acid, maleic acid and AMPS in a composition containing an alkali metal silicate. However, this reference does not disclose a composition or method for inhibiting formation of mixed inorganic deposits.

DE 3 743 739 discloses a dishwashing composition comprising carbonate or sulfate, sodium silicate and a copolymer made of (meth)acrylic acid, (meth)acrylamide and a sulfonated monomer (e.g. AMPS).

The problem addressed by this invention is to find a composition capable of reducing formation of mixed inorganic deposits.

### Statement of Invention

The present invention is directed to a phosphorus-free automatic dishwashing detergent composition comprising: (a) a polymer comprising polymerized residues of: (i) 62.5 to 85 wt% acrylic acid, (ii) 5 to 20% maleic acid and (iii) 10 to 30 wt% 2-acrylamido-2-methylpropanesulfonic acid (AMPS); and having M_{w} at least 2,000; and (b) carbonate and silicate in a weight ratio from 2.5:1 to 1:3, respectively, wherein the composition comprises from 10 to 90 wt% total carbonate and silicate.

### Detailed Description

All percentages are weight percentages (wt%), and all temperatures are in °C, unless otherwise indicated. Weight average molecular weights, M_{w}, are measured by gel permeation chromatography (GPC) using polyacrylic acid standards, as is known in the art. The techniques of GPC are discussed in detail in Modem Size Exclusion Chromatography, W. W. Yau, J. J. Kirkland, D. D. Bly; Wiley-Interscience, 1979, and in A Guide to Materials Characterization and Chemical Analysis, J. P. Sibilia; VCH, 1988, p. 81-84. The molecular weights reported herein are in units of daltons. As used herein the term "(meth)acrylic" refers to acrylic or methacrylic; the term "carbonate" to alkali metal or ammonium salts of carbonate, bicarbonate, percarbonate, sesquicarbonate; the term "silicate" to alkali metal or ammonium salts of silicate, disilicate, metasilicate; and the term "citrate" to alkali metal citrates. In some embodiments of the invention, the carbonates, silicates or citrates are sodium, potassium or lithium salts; alternatively sodium or potassium; alternatively sodium. The term "phosphorus-free" refers to compositions containing less than 0.5 wt% phosphorus (as elemental phosphorus), alternatively less than 0.2 wt%, alternatively less than 0.1 wt%, alternatively no detectable phosphorus.

The total weight of carbonate and silicate in the composition is from 10 to 90 wt% of the total weight of the composition. In some embodiments of the invention, total weight of carbonate and silicate is at least 15 wt%, alternatively at least 20 wt%, alternatively at least 25 wt%, alternatively at least 30 wt%, alternatively at least 35 wt%. In some embodiments, the total weight of carbonate and silicate is no more than 85 wt%, alternatively no more than 80 wt%, alternatively no more than 75 wt%, alternatively no more than 70 wt%, alternatively no more than 65 wt%, alternatively no more than 60 wt%. In some embodiments of the invention, the weight ratio of carbonate to silicate is no more than 2:1, alternatively no more than 1:1. In some embodiments, the weight ratio of carbonate to silicate is at least 1:2.5, alternatively at least 1:2, alternatively at least 1:1.5. In some embodiments of the invention, the composition further comprises an alkali metal citrate and/or aminocarboxylate. In some embodiments, the amount of alkali metal citrate is from 0.01 to 40 wt%, alternatively no more 35 wt%, alternatively no more than 30 wt%, alternatively no more than 25 wt%, alternatively no more than 20 wt%.

In some embodiments of the invention, the polymer comprises polymerized residues which are at least 65 wt% acrylic acid, alternatively at least 67.5 wt%, alternatively at least 70 wt%, alternatively at least 72.5 wt%. In some embodiments, the amount of acrylic acid residues in the polymer is no more than 85 wt%, alternatively no more than 82.5 wt%, alternatively no more than 80 wt%, alternatively no more than 77.5 wt%. In some embodiments of the invention, the maleic acid residues are at least 7.5 wt% of the polymer, alternatively at least 10 wt%, alternatively at least 12.5 wt%. In some embodiments, the amount of maleic acid residues is no more than 22.5%, alternatively no more than 20 wt%, alternatively no more than 17.5 wt%, alternatively no more than 15 wt%, alternatively no more than 12.5 wt%. Typically, the polymer is made by polymerizing maleic anhydride, which is hydrolyzed to the acid during the polymerization process. All references to maleic acid residues in the polymer include metal salts of maleic acid residues which would be present at pH values near or above the pKa of the carboxylic acid groups. In some embodiments of the invention, the amount of AMPS residues (including metal or ammonium salts) in the polymer is at least 12.5 wt%. In some embodiments, the amount of AMPS residues in the polymer is no more than 27.5 wt%, alternatively no more than 25 wt%, alternatively no more than 22.5 wt%, alternatively no more than 20 wt%, alternatively no more than 17.5 wt%. In some embodiments of the invention, the total amount of maleic acid and AMPS in the polymer is at least 15 wt%, alternatively at least 17 wt%, alternatively at least 19 wt%, alternatively at least 21 wt%, alternatively at least 23 wt%.

In some embodiments of the invention, the polymer contains no more than 5 wt% of esters of acrylic or methacrylic acid, alternatively no more than 2 wt%, alternatively no more than 1 wt%, alternatively no more than 0.5 wt%.

In some embodiments of the invention, the polymer has M_{w} of at least 4,000, alternatively at least 6,000, alternatively at least 8,000, alternatively at least 10,000, alternatively at least 12,000, alternatively at least 14,000. In some embodiments, M_{w} is no more than 300,000, alternatively no more than 200,000, alternatively no more than 100,000.

The polymer may be used in combination with other polymers useful for controlling insoluble deposits in automatic dishwashers, including, e.g, polymers comprising combinations of residues of acrylic acid, methacrylic acid, maleic acid or other diacid monomers, esters of acrylic or methacrylic acid including polyethylene glycol esters, styrene monomers, AMPS and other sulfonated monomers, and substituted acrylamides or methacrylamides.

The polymer of this invention may be produced by any of the known techniques for polymerization of acrylic monomers. In some embodiments of the invention, the initiator does not contain phosphorus. In some embodiments of the invention, the polymer contains less than 1 wt% phosphorus, alternatively less than 0.5 wt%, alternatively less than 0.1 wt%, alternatively the polymer contains no phosphorus. In some embodiments of the invention, polymerization is initiated with persulfate and the end group on the polymer is a sulfate or sulfonate. The polymer may be in the form of a water-soluble solution polymer, slurry, dried powder, or granules or other solid forms.

Other components of the automatic dishwashing detergent composition may include, e.g., surfactants, oxygen and/or chlorine bleaches, bleach activators, enzymes, foam suppressants, colors, fragrances, antibacterial agents and fillers. Typical surfactant levels depend on the particular surfactant used, typically from 0.1 wt% to 10 wt%, alternatively from 0.5 wt% to 5 wt%. Fillers in tablets or powders are inert, water-soluble substances, typically sodium or potassium salts, e.g., sodium or potassium sulfate and/or chloride, and typically are present in amounts ranging from 0 wt% to 75 wt%. Fillers in gel formulations may include those mentioned above and also water. Fragrances, dyes, foam suppressants, enzymes and antibacterial agents usually total no more than 5 wt% of the composition.

In some embodiments of the invention, the composition contains from 0.1 to 2 wt% of a hypochlorite salt, alternatively from 0.5 to 1.5 wt%. In some embodiments of the invention, the composition has a pH (at 1 wt% in water) of at least 10, alternatively at least 11.5; in some embodiments the pH is no greater than 13.

The composition can be formulated in any typical form, e.g., as a tablet, powder, monodose, sachet, paste, liquid or gel. The composition can be used under typical operating conditions for any typical automatic dishwasher. Typical water temperatures during the washing process preferably are from 20°C to 85°C, alternatively from 30°C to 70°C. Typical concentrations for the composition as a percentage of total liquid in the dishwasher preferably are from 0.1 to 1 wt%, alternatively from 0.2 to 0.7 wt%. With selection of an appropriate product form and addition time, the composition may be present in the prewash, main wash, penultimate rinse, final rinse, or any combination of these cycles.

In some embodiments of the invention, the composition comprises from 0.5 to 12 wt% of said polymer, alternatively from 1 to 10 wt%, alternatively from 2 to 8 wt%, alternatively from 3 to 7 wt%, alternatively from 3.5 to 6.5 wt%. In some embodiments of the invention, the weight ratio of polymer to the total amount of carbonate and silicate is no more than 1:2, alternatively no more than 1:3, alternatively no more than 1:4, alternatively no more than 1:5, alternatively no more than 1:6, alternatively no more than 1:7. In some embodiments of the invention, the weight ratio of polymer to the total amount of carbonate and silicate is at least 1:25, alternatively at least 1:20, alternatively at least 1:15, alternatively at least 1:10.

### Examples

Typical Polymer Preparation - To a two liter round bottom flask, equipped with a mechanical stirrer, heating mantle, thermocouple, condenser and inlets for the addition of monomer, initiator and chain regulator was charged 26.0 grams of maleic anhydride and 150 grams of deionized water. The mixture was set to stir and heated to 78°C (+/- 2°C). In the meantime, a monomer solution of 228.8 grams of glacial acrylic acid and 92.4 grams of 50% solution of sodium 2-acrylamido-2-methypropane sulfonic acid in water was added to a graduated cylinder, thoroughly mixed for addition to the flask. An initiator solution of 8.3 grams of sodium persulfate was dissolved in 30 grams of deionized water and added to a syringe for addition to the kettle. A chain regulator (CTA) solution of 18 grams of sodium metabisulfite dissolved in 45.5 grams of deionized water was added to a syringe for addition to the kettle. A chain regulator pre-charge solution was prepared by dissolving 0.73 grams of sodium metabisulfite in 5 grams of deionized water and set aside. A promoter solution of 3.88 grams of a 0.15% iron sulfate heptahydrate solution was added to a vial and set aside.

Once the kettle contents reached reaction temperature of 78°C, the promoter solution was added, followed by the sodium metabisulfite pre-charge solution. After the reaction temperature recovered to 78°C, the monomer, initiator and CTA solution feeds were begun simultaneously. The monomer feed rate was constant over 120 minutes. The CTA cofeed was added linearly over 105 minutes and the initiator cofeed added linearly over 125 minutes at 78°C.

At the completion of the feeds, 5 grams of deionized water was added to the monomer feed vessel, as rinse. The reaction was held for 15 minutes at 78°C. In the meantime, the chaser solution of 0.90 grams of sodium persulfate and 15 grams of deionized water was mixed and set aside.

At the completion of the hold, the above chaser solution was added linearly over 10 minutes and held for 15 minutes at 78°C.

At the completion of the final hold, cooling was begun with the addition of 100 grams of deionized water. At 50°C or below a solution of 168.9 grams of 50% sodium hydroxide was added to an addition funnel and slowly added to the kettle, controlling the exotherm to keep the temperature below 70°C. Finally, 1.9 grams of a scavenger solution of 35% hydrogen peroxide was added to the kettle. The reaction was then cooled and packaged.

The final polymer had a solids content of 43.68% (as measured in a forced draft oven at 150°C for 60 minutes). pH of the solution was 5.65 and final M_{w} as measured by Gel Permeation Chromatography was 16,872, and Mn was 3329. The residual monomer measured was <1 ppm acrylic acid, < 1 ppm maleic acid, and 839 ppm fumaric acid.

Polymer Testing - All polymers were tested for scale reduction by incorporating them at 1 g with sodium carbonate and/or sodium disilicate (BRITESIL H 20, PQ Corp.), and in some cases citrate, as indicated and washing glasses for 5 cycles in a Kenmore dishwasher (solids added to pre-wash and main wash cycles) using water with 400 ppm hardness (2:1 Ca⁺²:Mg⁺²) at 130 °F (54.4 °C) with no food soil. Glasses were evaluated after 1, 3 and 5 cycles using the scale from ASTM method 3556-85 (1=clean, 5=heavy film).

Table 1 presents results obtained using the polymer with a mixture of 4 g sodium carbonate and 6 g sodium disilicate.

**Table 1**

| polymer | M_{w} | filming scores | | |
|---|---|---|---|---|
| | | 1 cycle | 3 cycles | 5 cycles |
| none | - | 1.6 | 4.1 | 4.9 |
| 90 AA/10 Mal (phosphono end group, 1.7 wt% P) (comparative) | 1.9K | 1.7 | 2.1 | 2.7 |
| 100 AA (comparative) | 4.5K | 1.9 | 2.8 | 3.6 |
| 75 AA/10 Mal/15 AMPS | 15.9K | 1.8 | 2.0 | 2.1 |
| 65 AA/20 Mal/15 AMPS | 12K | 2.1 | 2.6 | 3.0 |
| 75 AA/10 Mal/15 AMPS | 16.9K | 1.3 | 2.1 | 3.1 |

| | | | | |
|---|---|---|---|---|
| Note: AA=acrylic acid; Mal=maleic acid; AMPS=2-acrylamido-2-methylpropanesulfonic acid, sodium salt; numbers associated with these abbreviations indicate wt% in the polymer. In M_{w}, K=1000, i.e., 1.9K=1,900 | | | | |

The polymers used in the present composition (below the double lines) perform better than the comparative polymers, sometimes with the exception of the first comparative entry, which contains phosphorus and thus is not desirable in a "phosphorus-free" formulation.

Table 2 presents results obtained using the polymer with a mixture of 4 g sodium carbonate, 6 g sodium disilicate and 2 g sodium citrate.

**Table 2**

| polymer | M_{w} | filming scores | | |
|---|---|---|---|---|
| | | 1 cycle | 3 cycles | 5 cycles |
| none | - | 1.9 | 3.8 | 5.0 |
| 90 AA/10 Mal (phosphono end group) (comparative) | 1.9K | 1.3 | 1.7 | 1.9 |
| 72 AA/28 AMPS (comparative) | 12K | 1.6 | 3.4 | 4.6 |
| 75 AA/10 Mal/15 AMPS | 15.9K | 1.4 | 1.6 | 2.5 |
| 75 AA/10 Mal/15 AMPS | 16.9K | 1.3 | 1.6 | 1.9 |

Table 3 presents results obtained using the polymer with 4 g sodium carbonate alone. This table is comparative because no silicate is present in these tests.

**Table 3 (comparative)**

| polymer | M_{w} | filming scores | | |
|---|---|---|---|---|
| | | 1 cycle | 3 cycles | 5 cycles |
| none | - | 2.7 | 5 | 5+ |
| 100 AA | 4.5K | 1.4 | 1.7 | 1.9 |
| 72 AA/28 AMPS | 12K | 1.6 | 1.7 | 1.8 |
| 75 AA/10 Mal/15 AMPS | 16.9K | 1.4 | 1.7 | 1.8 |

Table 4 presents results obtained using the polymer with 6 g sodium disilicate alone. This table is comparative because no carbonate is present in these tests.

**Table 4 (comparative)**

| polymer | M_{w} | filming scores | | |
|---|---|---|---|---|
| | | 1 cycle | 3 cycles | 5 cycles |
| none | - | 2.3 | 2.1 | 2.8 |
| 100 AA | 4.5K | 2.1 | 2.3 | 3.2 |
| 72 AA/28 AMPS | 12K | 2.0 | 1.8 | 1.8 |
| 75 AA/10 Mal/15 AMPS | 16.9K | 2.4 | 2.1 | 2.4 |

Table 5 presents results obtained using the polymer with a mixture of 2 g sodium carbonate and 8 g sodium disilicate.

**Table 5 (comparative)**

| polymer | M_{w} | filming scores | | |
|---|---|---|---|---|
| | | 1 cycle | 3 cycles | 5 cycles |
| none | - | 1.9 | 2.3 | 3.6 |
| 100 AA | 4.5K | 1.6 | 2.1 | 2.8 |
| 72 AA/28 AMPS | 12K | 1.5 | 1.8 | 2.4 |
| 75 AA/10 Mal/15 AMPS | 16.9K | 2.0 | 2.6 | 3.1 |

Table 6 presents results obtained using the polymer with a mixture of 8 g sodium carbonate and 2 g sodium disilicate.

**Table 6 (comparative)**

| polymer | M_{w} | filming scores | | |
|---|---|---|---|---|
| | | 1 cycle | 3 cycles | 5 cycles |
| none | - | 1.7 | 4.6 | 5+ |
| 100 AA | 4.5K | 1.8 | 3.8 | 4.7 |
| 72 AA/28 AMPS | 12K | 2.1 | 5+ | 5++ |
| 75 AA/10 Mal/15 AMPS | 16.9K | 1.7 | 3.5 | 5+ |

Table 7 presents results obtained using the polymer with a mixture of 6 g sodium carbonate and 2 g sodium disilicate.

**Table 7 (comparative)**

| polymer | M_{w} | filming scores | | |
|---|---|---|---|---|
| | | 1 cycle | 3 cycles | 5 cycles |
| none | - | 1.2 | 4.5 | 5 |
| 100 AA | 19.9K | 1.2 | 2.9 | 4.1 |
| 70 AA/30 MAA | 19.6K | 1.7 | 5 | 5+ |
| 40 Mal/60 MAA | 19.5K | 1.4 | 2.5 | 4.3 |
| 85 AA/10 Mal/5 AMPS | 18.9K | 1.3 | 2.4 | 4.7 |
| 80 AA/10 Mal/10 AMPS | 16.7K | 1.3 | 3.1 | 4.4 |
| 75 AA/10 Mal/15 AMPS | 16.9K | 1.4 | 4.8 | 5+ |
| 70 AA/10 Mal/20 AMPS | 19.0K | 1.3 | 4.5 | 5+ |
| 65 AA/10 Mal/25 AMPS | 19.0K | 1.6 | 4.4 | 5+ |

Table 8 presents results obtained using the polymer with a mixture of 1.5 g sodium carbonate and 6 g sodium disilicate.

**Table 8 (comparative)**

| polymer | M_{w} | filming scores | | |
|---|---|---|---|---|
| | | 1 cycle | 3 cycles | 5 cycles |
| none | - | 1.1 | 3.7 | 5.0 |
| 100 AA | 19.9K | 1.5 | 2.7 | 4.8 |
| 70 AA/30 MAA | 19.6K | 2.2 | 3.3 | 3.8 |
| 40 Mal/60 MAA | 19.5K | 1.6 | 2.8 | 3.5 |
| 85 AA/10 Mal/5 AMPS | 18.9K | 1.2 | 3.1 | 3.7 |
| 80 AA/10 Mal/10 AMPS | 16.7K | 1.2 | 3.4 | 4.0 |
| 75 AA/10 Mal/15 AMPS | 16.9K | 1.1 | 2.4 | 3.1 |
| 70 AA/10 Mal/20 AMPS | 19.0K | 1.2 | 3.1 | 4.2 |
| 65 AA/10 Mal/25 AMPS | 19.0K | 1.3 | 2.5 | 4.4 |

## Claims

1. A automatic dishwashing detergent composition containing less than 0.5 wt % phosphorus comprising:
(a) a polymer comprising polymerized residues of: (i) 62.5 to 85 wt% acrylic acid, (ii) 5 to 20% maleic acid and (iii) 10 to 30 wt% 2-acrylamido-2-methylpropanesulfonic acid; and having M_{w} at least 2,000; and
(b) carbonate and silicate in a weight ratio from 2.5:1 to 1:3 respectively, wherein the composition comprises from 10 to 90 wt% total carbonate and silicate.

2. The composition of claim 1 in which said polymer comprises polymerized residues of:
(i) 62.5 to 80 wt% acrylic acid, (ii) 7.5 to 15% maleic acid and (iii) 10 to 20 wt% 2-acrylamido-2-methylpropanesulfonic acid.

3. The composition of claim 1 in which the composition comprises from 15 to 50 wt% total carbonate and silicate.

4. The composition of claim 1 in which the composition comprises carbonate and silicate in a weight ratio from 1.5:1 to 1:3.

5. The composition of claim 1 in which said polymer contains less than 0.5 wt% phosphorus.

6. The composition of claim 1 in which said polymer comprises polymerized residues of:
(i) 65 to 80 wt% acrylic acid, (ii) 7.5 to 15% maleic acid and (iii) 10 to 20 wt% 2-acrylamido-2-methylpropanesulfonic acid; the composition comprises from 15 to 50 wt% total carbonate and silicate; and carbonate and silicate in a weight ratio from 1.5:1 to 1:3.

7. The composition of claim 6 in which said polymer has M_{w} at least 8,000.

8. The composition of claim 7 in which said polymer comprises polymerized residues of:
(i) 70 to 80 wt% acrylic acid, (ii) 7.5 to 12.5 wt% maleic acid and (iii) 12.5 to 17.5 wt% 2-acrylamido-2-methylpropanesulfonic acid.

9. The composition of claim 8 in which said polymer contains less than 0.5 wt% phosphorus.

10. The composition of claim 9 further comprising at least 0.1 wt% of a hypochlorite salt and having a pH of at least 11.5.

## Patentansprüche

1. Eine Spülmittelzusammensetzung für Geschirrspülmaschinen, die weniger als 0,5 Gew.-% Phosphor enthält, welche Folgendes beinhaltet:
(a) ein Polymer, das polymerisierte Reste von Folgendem beinhaltet: (i) 62,5 bis 85 Gew.-% Acrylsäure, (ii) 5 bis 20 % Maleinsäure und (iii) 10 bis 30 Gew.-% 2-Acrylamido-2-methylpropansulfonsäure; und ein M_{w} von mindestens 2000 aufweist; und
(b) Carbonat und Silicat in einem Gewichtsverhältnis von jeweils 2,5:1 bis 1:3, wobei die Zusammensetzung insgesamt von 10 bis 90 Gew.-% Carbonat und Silicat beinhaltet.

2. Zusammensetzung gemäß Anspruch 1, wobei das Polymer polymerisierte Reste von Folgendem beinhaltet:
(i) 62,5 bis 80 Gew.-% Acrylsäure, (ii) 7,5 bis 15 % Maleinsäure und (iii) 10 bis 20 Gew.-% 2-Acrylamido-2-methylpropansulfonsäure.

3. Zusammensetzung gemäß Anspruch 1, wobei die Zusammensetzung insgesamt von 15 bis 50 Gew.-% Carbonat und Silicat beinhaltet.

4. Zusammensetzung gemäß Anspruch 1, wobei die Zusammensetzung Carbonat und Silicat in einem Gewichtsverhältnis von 1,5:1 bis 1:3 beinhaltet.

5. Zusammensetzung gemäß Anspruch 1, wobei das Polymer weniger als 0,5 Gew.-% Phosphor enthält.

6. Zusammensetzung gemäß Anspruch 1, wobei das Polymer polymerisierte Reste von Folgendem beinhaltet:
(i) 65 bis 80 Gew.-% Acrylsäure, (ii) 7,5 bis 15 % Maleinsäure und (iii) 10 bis 20 Gew.-% 2-Acrylamido-2-methylpropansulfonsäure; wobei die Zusammensetzung insgesamt von 15 bis 50 Gew.-% Carbonat und Silicat beinhaltet; und Carbonat und Silicat in einem Gewichtsverhältnis von 1,5:1 bis 1:3.

7. Zusammensetzung gemäß Anspruch 6, wobei das Polymer ein M_{w} von mindestens 8000 aufweist.

8. Zusammensetzung gemäß Anspruch 7, wobei das Polymer polymerisierte Reste von Folgendem beinhaltet:
(i) 70 bis 80 Gew.-% Acrylsäure, (ii) 7,5 bis 12,5 Gew.-% Maleinsäure und (iii) 12,5 bis 17,5 Gew.-% 2-Acrylamido-2-methylpropansulfonsäure.

9. Zusammensetzung gemäß Anspruch 8, wobei das Polymer weniger als 0,5 Gew.-% Phosphor enthält.

10. Zusammensetzung gemäß Anspruch 9, die ferner mindestens 0,1 Gew.-% eines Hypochloritsalzes beinhaltet und einen pH von mindestens 11,5 aufweist.

## Revendications

1. Une composition de détergent pour lave-vaisselle automatique contenant moins de 0,5 % en poids de phosphore comprenant:
(a) un polymère comprenant des résidus polymérisés de : (i) entre 62,5 et 85 % en poids d'acide acrylique, (ii) entre 5 et 20 % d'acide maléique et (iii) entre 10 et 30 % en poids d'acide 2-acrylamido-2-méthylpropanesulfonique ; et présentant une Mᵣ d'au moins 2 000 ; et
(b) du carbonate et du silicate dans un rapport en poids compris entre 2,5/1 et 1/3, respectivement, la composition comprenant entre 10 et 90 % en poids de carbonate et de silicate au total.

2. La composition de la revendication 1 dans laquelle ledit polymère comprend des résidus polymérisés de :
(i) entre 62,5 et 80 % en poids d'acide acrylique, (ii) entre 7,5 et 15 % d'acide maléique et (iii) entre 10 et 20 % en poids d'acide 2-acrylamido-2-méthylpropanesulfonique.

3. La composition de la revendication 1, la composition comprenant entre 15 et 50 % en poids de carbonate et de silicate au total.

4. La composition de la revendication 1, la composition comprenant du carbonate et du silicate dans un rapport en poids compris entre 1,5/1 et 1/3.

5. La composition de la revendication 1 dans laquelle ledit polymère contient moins de 0,5 % en poids de phosphore.

6. La composition de la revendication 1 dans laquelle ledit polymère comprend des résidus polymérisés de :
(i) entre 65 et 80 % en poids d'acide acrylique,
(ii) entre 7,5 et 15 % d'acide maléique et
(iii) entre 10 et 20 % en poids d'acide 2-acrylamido-2-méthylpropanesulfonique ; la composition comprenant entre 15 et 50 % en poids de carbonate et de silicate au total ; et du carbonate et du silicate dans un rapport en poids compris entre 1,5/1 et 1/3.

7. La composition de la revendication 6 dans laquelle ledit polymère présente une Mᵣ d'au moins 8 000.

8. La composition de la revendication 7 dans laquelle ledit polymère comprend des résidus polymérisés de :
(i) entre 70 et 80 % en poids d'acide acrylique, (ii) entre 7,5 et 12,5 % en poids d'acide maléique et (iii) entre 12,5 et 17,5 % en poids d'acide 2-acrylamido-2-méthylpropanesulfonique.

9. La composition de la revendication 8 dans laquelle ledit polymère contient moins de 0,5 % en poids de phosphore.

10. La composition de la revendication 9 comprenant de plus au moins 0,1 % en poids d'un sel hypochlorite et présentant un pH d'au moins 11,5.
